

# United States Patent [19]

Baukal et al.

[11] 3,923,969

[45] Dec. 2, 1975

[54] CARRIER SYSTEM FOR A DRUG WITH SUSTAINED RELEASE

3,148,124 9/1964 Gaunt ..... 424/22

[75] Inventors: Werner Baukal, Kronberg, Taunus; Heinz-Joachim Kinkel, Schwalbach, Taunus; Erich Robens, Friedrichsdorf; Gerhard Walter, Steinbach, all of Germany

Primary Examiner—Shep K. Rose  
Attorney, Agent, or Firm—Christen & Sabol

[73] Assignee: Battelle-Institut e.V., Frankfurt am Main, Germany

[57] ABSTRACT

[22] Filed: June 12, 1973

A carrier system for a drug which allows the sustained and prolonged release of the drug which is comprised of (i) a porous carrier material which is insoluble or only slightly soluble in the body, which is in compacted form or powder form and which contains cavities which are connected to the outer surface by narrow pore necks, the mean diameters of the cavities in section being over twice as large as the mean internal widths of the necks of the pores, and the internal width of the necks of the pores being preponderantly less than 0.1  $\mu$ m, and (ii) a drug or pharmaceutically active substance is embedded or contained in the cavities.

[21] Appl. No.: 369,404

[52] U.S. Cl. ..... 424/19; 424/22; 424/23;  
424/357

[51] Int. Cl.<sup>2</sup> ..... A61K 27/12

[58] Field of Search ..... 424/19-23,  
424/357

## [56] References Cited

### UNITED STATES PATENTS

2,038,694 4/1936 Wiggins ..... 424/23

1 Claim, No Drawings

## CARRIER SYSTEM FOR A DRUG WITH SUSTAINED RELEASE

### BACKGROUND OF THIS INVENTION

#### 1. Field of this Invention

The invention relates to a carrier, depot or bonding system for a drug which allows sustained release of the drug and which can be administered orally, externally or by implantation. The carrier material consists of physiologically innocuous, inorganic or organic materials which are totally or almost non-reabsorbable in the body. For its properties as a carrier of active pharmaceutical substances what is decisive is the special porous structure. It comprises so-called inkwell pores, i.e. it contains cavities connected to the outer surface of the bonding substance by passages (pore necks) which are narrow in relation to their diameters. The drug is embedded in the cavities.

#### 2. Prior Art

Sustained release preparations make it possible for the dosage of a drug to be accurately controlled over a long period of time and for a plurality of active substances to be released on a set time schedule. A number of methods of obtaining sustained release are already known. For example, the drug may be enclosed in a capsule which will dissolve in the body after a certain amount of time or which allows the drug to diffuse through its porous wall. In the case of microincapsulation, the drug is enclosed in a large number of very small membrane capsules. Tablets may be coated with lacquers to achieve delayed release. The drug may be suspended in water, oil or buffer solutions. The drug may be etherified or esterified to put it in a form in which it is difficult to reabsorb. If the drug is applied as a crystal suspension or a crystal implant, its release will be delayed because its surfaces will be small relative to the amorphous substance. Absorption of the drug in carrier materials which can swell, such as gelatin, cellulose or certain plastics also delay release. If the drug is bonded by adsorption to large surfaces, release will be slow due to the low speed of desorption, as, e.g., in the case of the adsorbate inoculate or vaccine, a result of admixture with aluminium hydroxide. If a powdered drug is compressed together with powdered plastics, a porous tablet will form in which the plastic material will partly cover the surface of the powdered drug and will delay its release (see British Pat. No. 808,014, German Pat. No. 1,201,950 and U.S. Pat. No. 3,279,996).

### BROAD DESCRIPTION OF THIS INVENTION

The problem solved by this invention was the development of a carrier, bonding or depot system for sustained release preparations which has the following advantages as compared with known carrier means: (1) it is adapted to incorporate various solid or liquid drugs, independent of their chemical nature, solubility and mechanical or thermal stability, and (2) the rate at which the drug is released from the carrier substance into the body remains constant over a selectable period of time independently of the amount of stored drug or varies in accordance with a schedule or program.

According to this invention, these requirements are fulfilled when the drug, medicament or pharmaceutically active substance is incorporated in a porous carrier substance which is insoluble or only slightly soluble in the body (human and/or animal) and when the pores of the carrier substance each have an inkwell shape. In

the literature (see, e.g., G.J. Gregg and K.S.W. Sing, "Adsorption, Surface Area and Porosity": London, Academic Press (1967), page 145 ff), inkwell pores are pores which, in the simplest case, comprise a cavity which opens towards the outside through a narrow neck. With these pores two essential parameters can be chosen independently of one another: (i) the volume of the cavity and (ii) the dimensions (internal width and length) of the neck of the pore. If the volume of the neck is small relative to the volume of the cavity, the amount which can be stored in the pores will depend virtually only on the volume of the cavity, while the timing of the release or temporal course of delivery into a surrounding medium will be affected predominately by the dimensions of the pore neck. The pore systems having inkwell pores which are used in this invention are composed of a plurality of pores of different shapes and sizes, and the cavities are frequently interconnected and open to the outer surface of the porous substance through a plurality of necks. Pore systems of such very complex construction can be described, in their adsorption behavior action, as an inkwell shape, if the diameters of the cavities are on the average more than twice as large as the associated pore necks. This invention involves or uses only those inkwell pores in which the necks are within the micro- and mesopore range, i.e., having internal widths or diameters of less than  $0.1 \mu m$  down to the diameter of only a few atoms diameters (see, e.g., D.H. Everett and R.H. Ottewill, (eds.), "Surface Area Determination" London, Butterworths (1970) page 63).

For the sustained release preparation according to this invention, a porous carrier material which is insoluble or only slightly soluble in the body is used. The dimensions of the pores in such a material is virtually invariable during the period or time of application, so the rate at which the stored drug is discharged (rate of delivery) remains constant so long as the concentration in the cavities does not drop.

After the application or taking of a sustained release preparation comprised of an insoluble carrier substance having inkwell pores and a drug incorporated therein, body fluid first enters the pores and dissolves the drug or mixes with it. The drug then diffuses outwardly via the pore necks filled with body fluid while more body fluid diffuses inwardly. The drug initially has saturation concentration in the cavities and almost zero concentration outside (in the body). With regard to the timing of the release of drug when the starting processes are over, one should distinguish between the following two cases:

1. The active substance is soluble only to a limited extent in the body fluid and forms a separate phase. In this case the concentration of active substance in the solution in the cavity, and with it the rate of release or delivery, will remain constant until the separate phase has disappeared. It will then decrease.
2. The active substance can be mixed with the body fluid in any ratio. The concentration of active substance and the rate of release or delivery will then decrease continuously. The neck of the pore acts as a resistance to or check on the flow of active substance and lengthens the period of release.

If the dimensions of the necks in the pore system vary widely, the pores with short and wide necks will empty first, while the concentration in the other pores will remain constant for longer. The rate of release from such a pore system will decrease with the passage of time.

With a suitable combination, provision can be made for the drugs to be released with any timing, e.g., in approximately linear progression. By mixing pore systems of different types, filled with different active substances, programmed release of combinations of active substances also are obtained.

The rate of discharge from a carrier system with inkwell pores can be estimated from their dimensions, as demonstrated by the following example. The composition is taken to be a tablet with a volume of  $100 \text{ mm}^3$  less the cavity volume  $V$  of  $10 \text{ mm}^3$ . The cavities are connected to the surface by  $a = 10^8$  not very different pore necks with a mean cross-sectional area of  $A = 10 \text{ nm}^2$  and a mean length of  $0.1 \mu\text{m}$ . The concentration of active substance in the cavities when the starting processes are over is  $c_2 = 0.1 \mu\text{mol/mm}^3$ , while the concentration  $c_1$  in the body in the vicinity of the tablet is 0. Assuming a coefficient of diffusion of  $D = 10^{-9} \text{ m}^2 \text{ s}^{-1}$ , then according to Fick's Law the following is obtained, in simplified form, for the rate of release  $\dot{n}$  (sec, e.g., C.D. Hodgman, "Handbook of Chemistry and Physics", 44 ed., Cleveland, Chemical Rubber Publishing 1961, page 2274), :

$$N = - D a A \frac{C_2 - C_1}{1} = 10^{-9} \text{ mol.s}^{-1}$$

If the active substance has a molecular weight  $M$  of 200 and a density  $\delta$  of  $10^6 \text{ g.m.}^{-3}$ , then, assuming that the concentrations remain constant (Case 1), the period of discharge  $t$  will be:

$$t = \frac{n}{\dot{n}} = \frac{V \rho}{m \dot{n}} = 15 \text{ h}$$

The rate of discharge of active substance would accordingly remain constant for longer than  $\frac{1}{2}$  day, given low solubility.

With  $a = 10^{-6}$  and  $1 - 10 \mu\text{m}$ , one would obtain  $\dot{n} = 10^{-12} \text{ mol.s}^{-1}$  and a period of release  $t$  of 1.6 years.

Solids with an inkwell pore structure are known, they are used, for example, as adsorbents, catalysts or catalyst carriers. Suitable materials which can be used as the carrier material having an inkwell pore structure include oxides, ceramic and metallic materials and plastics which are physiologically innocuous. The preparations may be used as a powder or in a compact or compacted form, such as, tablet form.

Oxides such as silicon oxide, aluminium oxide, zirconium oxide, etc., can be prepared in highly porous form from the corresponding hydroxide gel by dehydration and drying at an elevated temperature (see, e.g., R.E. Kirk and D.F. Othmer, "Encyclopedia of Chemical Technology", Vol. 12, page 345 ff., New York, Interscience Publishers (1954); and E. Robens and G. Sandstede, "Z. Instrumentenkunde" 75 (1967), page 177). In another process (see K.S. Mazdiyasny, C.T. Lynch and J.S. Smith, J. Am. Ceramic Soc. 48 (1965), pages 372 - 375) alcoholates dissolved in organic solvents are converted, by hydrolysis and subsequent drying, into oxides with crystallites and pores in the sub-micron range.

Metallic and ceramic substances as well as plastics can be sintered together to form porous bodies by compressing powders, with a simultaneous or subsequent heat treatment. Porous structures of the desired type can be obtained by thermal disintegration of hydrates

or salts, e.g., in the thermal decomposition of nickel formate dihydrate (P.G. Fox, J. Ehretsmann and C.E. Brown, J. Catalysis 20 (1971), pages 67 - 73). The Raney process may be used to prepare metallic powders of very high micro-porosity. A metal alloy is first produced and one component of the alloy is then dissolved out. The remaining metal re-crystallizes, and micro-crystallites and corresponding pore systems are formed (see, e.g., H. Krupp, H. Rabenhorst, G. Sandstede, G. Walter and R. McJones, J. Elektrochemical Soc. 109 (1962), pages 553 - 557). Porous plastics can be made by various, already-known methods, e.g., by using one of the freeze drying techniques. In the processes mentioned herein, the pore structure can be modified by varying the manufacturing conditions.

The active substance may be deposited by steeping the bonding material in the liquid or molten drug. It may be necessary first to cleanse the material of substances (such as water) which have been embedded in the cavities during manufacture. This can be done, e.g., by drying under vacuum at an elevated temperature. Solid drugs may be dissolved and incorporated or placed in the bonding material by steeping the latter in the solution. The solvent can then be removed by vaporization. If the drug is vaporizable or sublimable, it may be deposited or placed in the cavities by condensation out of the gas phase. Finally, the drug may be mixed with the starting materials before the preparation of the carrier material. As the carrier material is made, the drug becomes enclosed in the pores which are formed.

Preparations made in this way can be used in powder form. The powder may be processed as an emulsion in a liquid in which the drug is insoluble or compressed into tablets. The carrier material in pellet or tablet form may be coated in a known manner with lacquers in order to achieve a further delay in the action of the drug.

As used herein the term drug includes medicaments, drugs, pharmaceutically active substances, etc.

The drug can be, for example: laxatives, such as, oxyphenisatin acetate; vitamins and nutrients; parasympatholytics, such as homatropine methylbromide or phenobarbital; hormones; steroids; anti-infectives; analgesics, such as, phenacetin, aspirin and caffeine; narcotics; anesthetics; sedatives and tranquilizers, such as, chlordiazepoxide HCl and diazepam; antihallucinatory agents; sympathomimetics; hypo-allergenic agents; antigens; antihistamines, such as, bromodiphenhydramine hydrochloride, methapyrilene fumarate and chlorpheniramine maleate; vasoconstrictors; antibiotics; enzymes; anticoagulants, vasodilators; lipotropic agents; cerebral stimulants; bronchodilators; muscle relaxants; diuretics; etc.

The carrier material consists of physiologically harmless inorganic or organic materials which cannot be absorbed or only very slightly absorbed in the body. Its special porous structure is critical for its use as a carrier of pharmaceutically active ingredients. It contains so-called inkwell pores, that is to say it contains cavities or hollow spaces, which are connected by channels (necks of the pores), which are narrow in relation to their diameter of the main cavity bodies, with the outside surface of the carrier material. The drug is housed in the hollow spaces.

## DETAILED DESCRIPTION OF THIS INVENTION

In the following examples and throughout the rest of this document, all parts, percentages and ratios are on a weight basis unless otherwise stated or obviously so to one ordinarily skilled in the art.

## EXAMPLE 1

## Benzoic acid in silica gel

An excess quantity of waterglass solution was stirred drop by drop into dilute hydrochloric acid at 50°C. A jelly formed, which was washed free of electrolyte and dried first at 100°C., then at 300°C. A piece of the resultant lumps of silica gel was de-gassed under vacuum and, again under vacuum, impregnated with molten benzoic acid (as a sample drug). The lump was then compressed in polyethylene powder in such a way that the silica gel was completely sheathed with a porous film of polyethylene. The tablet was put into water and the timing of the variation in conductivity resulting from the escape of benzoic acid was measured. A uniform increase in conductivity was observed over several hours.

## EXAMPLE 2

## 1-Propyl-1-cyclohexyl-2-methylaminopropane-hydrochloride in aluminium oxide

By the method of Mazdyasni, Lynch and Smith, aluminium-iso-propylate was dissolved in benzene, and a mixture of water and iso-propanol were added dropwise while stirring. Both mixtures contained the drug almost to the point of saturation. The jelly which formed was dried at 100°C. As in Example 1 the rate of

35

discharge was ascertained by measuring the conductivity, and the lump disintegrated into small particles. As first there was a strong discharge of the drug, which changed to a slow discharge after about a quarter of an hour. A constant rate of discharge could be observed for 2 days.

The initial strong discharge was decreased by washing and then drying the lump of the preparation.

What is claimed is:

10. 1. A carrier system for a drug which allows the sustained and prolonged release of the drug which consists of
  - i. a porous carrier aluminium oxide material which is insoluble or only slightly soluble in the body which is in dried jelly lump form which disintegrates into small particles and which contains inkwell pore cavities which are connected to the outer surface by narrow pore necks, the mean diameters of the inkwell pore cavities in section being over twice as large as the mean internal widths of the necks of the inkwell pores, and the internal width of the necks of the inkwell pores being preponderantly less than 0.1  $\mu\text{m}$  and
  15. ii. a drug or pharmaceutically active substance which is embedded or contained only in said inkwell pore cavities, and which jelly has been formed by stirring together dropwise a mixture of aluminum isoproponate dissolved in benzene and a mixture of water and isopropanol, both mixtures containing the drug almost to the point of saturation, and drying the jelly which formed, to a lump which disintegrates into small particles.

\* \* \* \* \*

40

45

50

55

60

65